

Nov. 11, 1930.

L. H. MARSHALL

1,781,119

PROCESS OF PRODUCING MALLEABLE IRON CASTINGS

Filed April 27, 1928



FIG. 1.



FIG. 2



FIG. 3

## UNITED STATES PATENT OFFICE

LESLIE H. MARSHALL, OF COLUMBUS, OHIO, ASSIGNOR OF ONE-HALF TO ADIN A. GRUBB, OF COLUMBUS, OHIO

## PROCESS OF PRODUCING MALLEABLE-IRON CASTINGS

Application filed April 27, 1928. Serial No. 273,208.

The invention relates to improved methods of producing malleable iron castings and the invention has to do especially with the annealing treatment employed in the production of the castings.

One object of the invention is to provide an improved process of producing rust-proof malleable iron castings by which the time, labor and cost of production are reduced while the standard of quality is amply maintained.

Another object of the invention is the production of malleable iron castings having uniformly good machining qualities.

Various other objects which are more or less incidental or ancillary to those above noted will appear in the following description.

In the usual procedure for making malleable iron castings, the metal is first cast as white iron. In this condition the iron is hard and brittle and can be machined only by grinding. Such castings, with or without sand blasting or other definite cleaning operations, are then packed in annealing pots, either with or without a surrounding packing of gravel or other refractory material. If the castings are small and the pots not large, the packing material is sometimes omitted, but where the castings are large the packing material is usually employed to support the castings and prevent their distortion at the elevated temperatures of the annealing treatment. The packing material also tends to lessen oxidation of the castings during the heat treatment.

The annealing pots or boxes when packed with the castings in one or the other of the above described ways, are carried into the annealing furnace, said furnace is closed and the firing started. Commonly an open flame type of furnace is employed in which the flames and hot gases sweep from the combustion chamber through the annealing chamber over and around the annealing boxes and thence out through suitable flues.

To properly anneal the castings a very definite treatment is required. Thus they must be held at an elevated temperature, (1400° to 1800° F.) for a period of from one to six days. The higher the temperatures within

the stated range the shorter is the holding period. Then the temperature is allowed to fall not faster than 10° F. per hour until it has reached 1000° F. The doors of the furnace can then be opened and the annealing pots and their contents allowed to cool to room temperature. In commercial practice the total time of the annealing cycle may vary in different plants, from six to fourteen days.

It is evident from the above that the castings during the annealing treatment receive a severe and protracted exposure to oxidizing conditions. In spite of the protection afforded by the gravel packing, the castings have an oxidized surface as they come from the anneal and frequently as high as 1% or more of the castings are rendered worthless by such oxidation.

A very considerable percentage of the malleable iron produced is subjected to some rust-proofing process soon after it is annealed. Usually this process is that of hot dip galvanizing in which the castings are given a zinc coating by immersing them in a bath of molten zinc. The castings must be clean and free from oxide or scale in order to take satisfactory zinc coatings. Accordingly, it has been necessary because of the oxidized and scaly condition of the annealed castings as heretofore produced to subject them to pickling and sand blasting preparatory to galvanizing. This pickling and sand blasting treatment involves expenditure of considerable time, labor and materials and adds materially to the cost of the finished rust-proof casting.

Another disadvantage that flows from the method of annealing castings as heretofore practiced is the formation on the surface of the casting of a layer or skin of relatively tough metal. This tough skin, though not hard, renders machining operations difficult by gumming and clogging the cutting tool. I believe that the formation of this tough outer layer on the annealed castings is due to decarbonization of the surface metal by reason of the oxidizing conditions that maintain during the prolonged heat treatment. The structure of American or black heart

malleable cast iron, after the anneal, consists essentially of a matrix of soft iron through which is interspersed nodules of graphite. The presence of the graphite lowers the strength of the metal somewhat but it adds greatly to the ease with which the metal can be machined. With oxidizing conditions prevailing during the anneal, the carbon near the surface of the casting is oxidized away before the iron is materially attacked, with the result that an outer layer of skin of the casting of substantial thickness loses most of its graphite.

Again, the annealing process as heretofore practiced sometimes causes the formation of a relatively hard outside layer or skin on the castings, such castings having what the trade terms "a picture frame" fracture. In this case, an appreciable percentage of combined carbon is present in the exterior layer while the interior, or by far major portion of the casting, is free from combined carbon. I believe this condition is due to the fact that a certain amount of silicon, as well as some but not all of the carbon, is oxidized out of the surface layer during the anneal and that this diminution of silicon prevents the complete graphitization of the carbon. The ungraphitized carbon combined with the iron forms a very hard compound which, as previously stated, seriously interferes with the machining of the casting.

Both of the last two defects become especially noticeable when the castings have to be threaded on the surface. In such a case the machining is confined largely to the section having the undesirable structure and while the major part of the casting may be normal, the machining is just as difficult as it would be if the casting were unsatisfactory throughout. A striking example of such a case is to be found in malleable cast iron pipe fittings, of which a large tonnage is produced, where a considerable percentage of the surface of each casting is threaded.

As all three of the above described objections to the prior practice are due to the presence of oxidizing conditions during annealing of the castings, I have sought to devise a method of easily and effectively maintaining non-oxidizing and preferably slightly etching conditions through the prolonged annealing treatment, or at least while the temperatures are high enough to cause a substantial amount of oxidation of the castings. The non-oxidizing conditions should obtain certainly above 1000° F. and preferably above 700° F. To this end the process provides for the maintenance around the castings of an atmosphere of non-oxidizing and preferably slightly etching gas or vapor, during the heat treatment of the castings, or at least during the existence of oxidizing temperatures. This can be done in various

ways. For example, some at least of the advantages of the process can be attained by conducting the non-oxidizing gas or vapor as such into closed pots or boxes which hold the castings during the annealing heat treatment. However, a method which I prefer because of its marked simplicity and effectiveness is to introduce into the closed annealing pots containing the castings a substance adapted when heated to say 1000° F. or less to evolve a gas or vapor having the desired non-oxidizing properties. I prefer also to employ the atmosphere of a gas or vapor that is heavier than air and to use tight-bottomed annealing boxes so that in the early stage of the heat treatment the relatively heavy gas or vapor displaces any air present and forces it from the container through leakage openings around the top thereof. Various substances can be employed to furnish the gaseous or vaporous atmosphere, such, for example, as ferric chloride, ferrous sulphate, and bleaching powder. However, I have secured the best results with halogen compounds that volatilize before temperatures are reached at which the substantial oxidation of the castings can occur. In order that my invention and the method of practicing it may be clearly understood, I shall now describe preferred methods of proceeding, reference being had to the accompanying drawings in which suitable apparatus is diagrammatically shown.

In the drawings:

Fig. 1 is a vertical section through a stack of annealing pots or boxes filled with castings ready for the annealing heat treatment.

Fig. 2 shows diagrammatically a typical open flame furnace with a series of stacks of annealing pots arranged therein for the heat treatment.

Fig. 3 is a transverse section on the line 3, 3 of Fig. 2.

A preferred specific procedure employing the apparatus illustrated is as follows: White iron castings that are to be malleablized, having first been thoroughly cleaned by sand blasting, tumbling or other suitable method are packed as at 1, 1 in a tight-bottomed annealing pot or box 2 and all voids around and between the castings are filled with a packing 3 consisting of 95% to 98% of sand and the balance (5% to 2%) of ferric chloride, the percentages being by weight. The chloride may be anhydrous or commercial ferric chloride crystals ( $FeCl_3 \cdot 6H_2O$ ) may be used. I have made satisfactory use of a packing consisting of 98% silica sand of about 8 mesh size and 2% of commercial ferric chloride crystals crushed to one inch and smaller pieces. A substantial layer of this packing material is preferably placed over the topmost castings to prevent oxidizing gases sweeping in and reaching the surfaces

70

75

80

85

90

95

100

105

110

115

120

125

130

of the castings. If a single annealing pot or box is to be employed a metal cover should be used to close its top, but in the present instance the pot 2 is closed by the bottom of a second pot 2' placed upon the top of pot 2, the pots being provided at their upper edges with upwardly extending flanges to facilitate such stacking. The second pot 2' is packed with castings and packing material in the same manner as above described, and similarly a third pot 2" may be stacked upon the second pot and similarly packed with castings. The top pot is then closed with a suitable metal plate 4. To reduce flow of gases through the joints between the pots and between the top pot and its cover 4, said joints are sealed by lutings 5 of suitable material such as paste formed by mixing powdered flint and water. To facilitate handling, the pots are stacked upon a suitable base 6.

The annealing pots having been packed and stacked in the manner described, are placed in an annealing furnace, designated in its entirety by 7, as indicated in Figs. 2 and 3. Then, the furnace charging door 8 having been closed, heating of the furnace is begun. In the furnace shown heat is supplied by a powdered coal burner 9. The flames and hot combustion gases of the burner are projected into the furnace over and around the stack of annealing pots, the gases finally passing out of the furnace at points near the floor through ducts 10, 10 which lead to flues 11 which in turn communicate with a stack or other suitable draft means.

The furnace, heated in this manner, has its annealing chamber gradually brought up to some suitable temperature between 1400° F. and 1800° F. and there held for one to six days, according to the temperature, as previously explained. For example, a satisfactory procedure is to consume 25 hours in heating the furnace to a temperature of 1650° F. after which the temperature is held between 1600° F. and 1650° F. for 60 hours, and after that the furnace is allowed gradually to cool to a temperature of approximately 1000° F. over a period of 80 hours. The doors of the furnace are then opened and the pots and their contents allowed to cool to room temperature.

The castings thus treated when removed from the annealing pots, because of the non-oxidizing and etching conditions maintained therein, are found to be bright and clean in appearance and in an especially good condition for the application of zinc or other rust-proof coatings. Furthermore, because of the non-oxidizing conditions under which the castings have been annealed, the castings as they come from the anneal are not only bright and clean but are substantially free from superficial layers that are either tough or unduly hard, so that the castings have uniformly good machining qualities.

If the castings annealed in accordance with my process are to be left exposed to air for any considerable length of time, a day or more, before receiving a rust-proof coating, they should be washed in a caustic solution to remove or neutralize the traces of halide that remain on them. Otherwise they will tarnish. A suitable treatment consists in agitating the castings for five minutes in a hot (just below the boiling point) 10% aqueous solution of tri-sodium phosphate to which has been added one volume of "soluble oil" to 30 volumes of the aqueous solution. (The term "soluble oil" is used to denote an oil that will stay suspended or emulsified in water when mixed therewith.) The castings thus treated will be hot enough to dry themselves after the treatment if they are permitted to drain properly. Such castings will be clean in appearance and resist tarnish in the usual indoor atmosphere very well.

It is obvious that the process above described can be modified in various ways. As has been indicated, the time and temperature of the annealing heat treatment can be considerably varied. Also, as has been stated, use can be made of various other substances in place of the ferric chloride. For example, the ferric chloride of the foregoing specific example can be replaced by a similar amount of ferrous sulphate. However, the latter substance does not give an atmosphere that is as completely non-oxidizing as can be secured by the use of halogen compounds and I accordingly prefer to use the latter.

Some of these halogen compounds merely vaporize and thus displace any air present in the container, the vapors being heavier than the air. The vapors also react to some extent with any scale that may form on the casting and this slight etching effect tends further to insure clean castings at the end of the annealing treatment. Examples of halogen compounds that merely vaporize, at least in part, below 700° F. are aluminum chloride, antimony chloride, arsenic chloride, mercuric chloride, phosphorus trichloride, carbon tetrachloride, sulphur monochloride and bismuth chloride. Others of the halogen compounds liberate halogen gases on heating and they are therefore particularly suitable as the halogen gas has a somewhat stronger etching effect than the halide vapors above noted, as well as serving to displace any air present and affording a non-oxidizing atmosphere. Examples of this latter class of halogen compounds are gold (auric) chloride, ferric chloride, cupric chloride, phosphorous pentachloride, sulphur dichloride, sulphur tetrachloride and bleaching powder. Halogen compounds other than chlorides can be used. For example, anhydrous ferric bromide is operable in the process, though some of the other halogen compounds are preferable because of their lower cost. While the ferric chloride

of the specific example given can be replaced by an equivalent amount of any one of the other substances enumerated, I have found that, all things considered, the ferric chloride and the bleaching powder are the ones most suitable for my process. It is not necessary to closely control the amount (5%) of the ferric chloride or other substance used in place of it, the chief consideration being to have enough of the substance present to insure the desired atmosphere and this can be done by using the substance more or less in excess.

It is to be observed further that the halogen compound employed need not be introduced as such into the treating container. Thus, in the packing material there can be substituted for the 2% of ferric chloride, for example, 4% (by weight) of a mixture of equal amounts by weight of powdered ferric sulphate (calcined) and powdered sodium chloride. On heating the packing, these two compounds react to give ferric chloride and sodium sulphate. Any other known method of forming ferric chloride, by reaction within the packing, might be used.

However, this method of introducing the ferric chloride usually contaminates the packing, as with the sodium sulphate in the example just given, and this may be undesirable.

The packing material employed in the process can to advantage be used over and over again. It is desirable to have the vaporizable compound present in excess so as to insure non-oxidizing conditions. Some of the halide vapor material recondenses on the inert material of the packing and thus would be lost if the packing were not repeatedly used. It can be reused successfully if enough of the vaporizable compound is added after each treatment to make up for the loss in the last preceding anneal. The amount to be added can best be determined by trial, that is by making a series of runs adding various amounts of the vaporizable compound to the reused packing material and noting the minimum amount that prevents oxidation of the castings. I have found that where a packing containing 2% of commercial ferric chloride crystals is used, an addition of 1% of said crystals is enough to adapt the packing for reuse.

In some instances of trouble with castings having the "picture frame" type of fracture, I find it desirable to supplement the non-oxidizing atmosphere during the heat treatment by the addition of a small amount of finely divided ferro-silicon to the packing material. In my copending application Serial No. 242,838, filed December 27, 1927, I have described a method for forming silicon or silicon alloy coatings on iron or other articles. In that method a typical procedure is to surround the article to be coated with a packing comprising inert material, such as

gravel, and suitable percentages of a vaporizable halide, such for example as anhydrous ferric chloride, and of ferro-silicon, the latter and the halide preferably being in a finely divided state. The article thus packed is then subjected to a suitable heat treatment, usually at temperatures within the range of the malleablizing heat treatment herein described. Now, in the method of the present application, I find that by the addition to the packing material of a smaller amount of ferro-silicon than is employed in the coating process, while no appreciable coating of silicon or silicon alloy is formed on the casting, nevertheless the effect is to prevent loss of silicon from the casting and thus obviate the above described troubles which go with the "picture frame" fracture. To carry out this modification of the process it is ordinarily sufficient to add to the packing material containing the usual (above specified) amount of halide, 0.25% by weight of ferro-silicon (50% silicon), indeed I have found as little as 0.1% of 20 mesh ferro-silicon (50% silicon) to be sufficient for the purpose.

It is to be observed that if the packing material containing a halide is to be out of use for any extended period of time, it should be kept in a closed container, as it tends to pick up moisture from the air and deteriorate.

In cases where it may be feasible or expedient to provide the non-oxidizing atmosphere by introducing a non-oxidizing gas as such into the otherwise closed annealing pot or container, as mentioned in the earlier part of this specification, the halogens, viz., chlorine, bromine, iodine and fluorine are the most suitable non-oxidizing gases for the purpose; and of these gases chlorine is the cheapest and to be preferred. The pressure and rate at which the gas is passed into the container will best be determined by trial, the object being, of course, to secure the desired result with a minimum amount of the gas.

My improved method of annealing in a halogen atmosphere tends to loosen the adherent sand and scale found on the castings as they come from the mold. It is possible, therefore, to anneal castings just as they come from the foundry and dispense with the cleaning operation previous to packing them for the anneal. It is then usually necessary to give the annealed castings a slight amount of tumbling to remove the last traces of sand or scale.

It frequently happens that castings have sand burned into their surface in the casting process, making them difficult or impossible to clean. Some are of such shape that parts of the surface cannot be readily reached by the ordinary methods of cleaning. Such castings after being annealed in a halogen at-

mosphere can be easily cleaned by the usual methods.

In characterizing herein the gas or vapor in the annealing pots as "non-oxidizing", that term is of course used in its strict or limited sense indicating that the gas or vapor is of such a nature that it will not form a film of metallic oxides on the castings during the annealing process.

10 It will now be apparent that my process, especially in its preferred forms, affords an exceedingly simple and easily practiced method of avoiding the previously explained ill effects of oxidizing conditions during the 15 malleablizing treatment, and it will also be apparent that satisfactory rust-proofed malleable castings and machined malleable castings can be produced at lower cost by my improved method than by the prior methods.

20 While I have set forth some of the variations as to materials and procedure which may be followed in the carrying out of my invention, it should be understood that I have not attempted to point out all such variations but that the invention comprehends all such modifications within the scope of the appended claims. Since, as has been explained, use can be made in my process of either halogen compounds that merely vaporize or those that evolve halogen gas at or below iron oxidizing temperatures, for the sake of simplicity and to avoid multiplication of claims, I shall in the appended claims use the term "halogen gas" in a broad sense comprehending both halide vapor and halogen gas.

What I claim is:

1. The improvement in the art of producing malleable iron castings which consists in 40 subjecting white iron castings to a heat treatment at temperatures and for a period of time adapted to effect malleablization of said castings, and maintaining around said castings a non-oxidizing and etching gaseous atmosphere while the temperature of the heat treatment is above 1000° F.

2. The improvement in the art of producing malleable iron castings which consists in subjecting white iron castings to a heat treatment 50 at temperatures and for a period of time adapted to effect malleablization of said castings, and maintaining around said castings a non-oxidizing and etching gaseous atmosphere while the temperature of the heat treatment is above 700° F.

3. The improvement in the art of producing malleable iron castings which consists in subjecting white iron castings to a heat treatment 60 at temperatures and for a period of time adapted to effect malleablization of said castings, and maintaining around said castings a non-oxidizing atmosphere of halogen gas while the temperature of the heat treatment is above 1000° F.

65 4. The improvement in the art of produc-

ing malleable iron castings which consists in subjecting white iron castings to a heat treatment at temperatures and for a period of time adapted to effect malleablization of said castings, and maintaining around said castings a non-oxidizing atmosphere of halogen gas while the temperature of the heat treatment is above 700° F.

5. The improved process of producing malleable iron castings which includes enclosing white iron castings in a tight bottomed container together with a substance capable when heated to temperatures below 1000° F. of evolving a non-oxidizing and etching gas heavier than air, and subjecting the said container and its contents to a heat treatment at temperatures and for a period of time adapted to effect malleablization of said castings, whereby a non-oxidizing and etching atmosphere is maintained around the castings during the said heat treatment.

6. The improved process of producing malleable iron castings which includes enclosing white iron castings in a tight bottomed container together with a substance capable when heated to temperatures below 700° F. of evolving a non-oxidizing and etching gas heavier than air, and subjecting the said container and its contents to a heat treatment at temperatures and for a period of time adapted to effect malleablization of said castings, whereby a non-oxidizing and etching atmosphere is maintained around the castings during the said heat treatment.

7. The improved process of producing malleable iron castings which includes enclosing white iron castings in a tight bottomed container together with a substance capable when heated of evolving a non-oxidizing halogen gas heavier than air, and subjecting the container and its contents to a heat treatment at temperatures and for a period of time adapted to effect malleablization of said castings, whereby a halogen gas atmosphere is maintained around said castings during said heat treatment.

8. An improved process of producing malleable iron castings which comprises enclosing white iron castings in a container together with a solid packing material composed in part of a refractory substance and in part of a substance capable when heated of evolving a non-oxidizing and etching gas, and subjecting the container and its contents to heat treatment at temperatures and for a 120 period of time adapted to effect malleablization of said castings, whereby a non-oxidizing and etching atmosphere is maintained around the castings during the said heat treatment.

9. An improved process of producing 125 malleable iron castings which comprises enclosing white iron castings in a container together with a packing material composed in part of a refractory substance and in part of a substance capable, when heated, of evolving 130

- 5 a non-oxidizing halogen gas, and subjecting the container and its contents to heat treatment at temperatures and for a period of time adapted to effect malleabilization of said castings, whereby a non-oxidizing atmosphere is maintained around the castings during the said heat treatment.
- 10 10. An improved process of producing malleable iron castings which comprises enclosing white iron castings in a container together with a packing material composed in part of a refractory substance and in part of ferric chloride, and subjecting the container and its contents to heat treatment at temperatures and for a period of time adapted to effect malleabilization of said castings, whereby a non-oxidizing atmosphere is maintained around the castings during the said heat treatment.
- 15 11. An improved process of producing malleable iron castings which comprises enclosing white iron castings in a container together with a packing material composed in part of a substance capable, when heated, of evolving halogen gas and in part of ferro-silicon, and subjecting the container and its contents to heat treatment at temperatures and for a period of time adapted to effect malleabilization of said castings, whereby a non-oxidizing atmosphere is maintained around the castings and loss of silicon from the castings is obviated during the said heat treatment.
- 20
- 25
- 30
- 35

In testimony whereof, I hereunto affix my signature.

LESLIE H. MARSHALL.